

July 28, 1959

A. ZLETZ ET AL

2,896,406

ROCKET PROPULSION METHOD

Filed Feb. 16, 1953



INVENTORS:  
Alex Zletz  
Don R. Carmody

BY  
*Michael Dugney*  
ATTORNEY

## ROCKET PROPULSION METHOD

Alex Zletz, Park Forest, and Don R. Carmody, Crete, Ill., assignors to Standard Oil Company, Chicago, Ill., a corporation of Indiana

Application February 16, 1953, Serial No. 336,909

19 Claims. (Cl. 60—35.4)

This invention relates to the generation of gas. More particularly, it relates to reaction propulsion by the hypergolic reaction of a liquid fuel and a liquid oxidizer. Still more particularly, the invention relates to a method of rocket propulsion by the hypergolic reaction of a fuel and a hydrogen peroxide oxidizer, which materials spontaneously react to generate gas at high pressure and high temperature.

Reaction propulsion is now being used for many aerial purposes. For many uses it is necessary to operate with a fuel system which is not dependent on atmospheric oxygen. This fuel system may consist of a single self-contained propellant or it may consist of a separate fuel and a separate oxidizer, i.e., a bipropellant system.

In the bipropellant system the fuel and the oxidizer are introduced separately and essentially simultaneously into the combustion chamber of the reaction motor. The products of oxidation from the reaction of the fuel and the oxidizer are discharged through an orifice at the exit end of the combustion chamber and thereby produce the driving force. Because of the possibilities of electrical and/or mechanical failure of the auxiliary methods of ignition such as a spark or a hot surface, it is preferred to use a self-igniting fuel system. A fuel which is self-igniting, i. e., spontaneously combustible when contacted with an oxidizer, is known as a hypergolic fuel.

Temperature has an important effect on the hypergolic activity of fuels. The temperature at the earth's surface may vary from a high of about +125° F. to a low of as much as -65° F.; in general temperatures below about -20° or -30° F. are exceptional. Thus surface-to-air missiles or rocket-driven aircraft should be capable of operation when the temperature of the fuel and the oxidizer at the moment of initial contact in the combustion chamber of the rocket motor is on the order of -20° F. Temperatures at high altitudes are frequently on the order of -65° F. and are known to approach -100° F. Thus an air-to-air missile should be able to operate satisfactorily when the temperature of the fuel and the oxidizer at the moment of initial contact in the combustion chamber is on the order of -65° F.

The more common oxidizers are white fuming nitric acid, red fuming nitric acid and nitric acid-sulfuric acid mixtures. While these nitric acid oxidizers operate satisfactorily over a wide range of atmospheric temperatures they have important drawbacks. The nitric acid oxidizers are extremely corrosive; they have poor storage stability; they give off toxic gases; and special precautions must be taken by personnel who handle these oxidizers.

Concentrated aqueous hydrogen peroxide solutions have excellent storage stability and do not give off harmful gas. However, these aqueous hydrogen peroxide solutions such as 90% hydrogen peroxide have the disadvantage of comparatively high freezing points, e.g., 90% hydrogen peroxide solution freezes at +12° F. The freezing point of 80% hydrogen peroxide is -9° F., but the activity of this solution toward the prior art fuels

is markedly lower than the 90%  $H_2O_2$  solution. The freezing point of aqueous hydrogen peroxide solutions can be depressed by dissolving therein inorganic salts, preferably ammonium nitrate. Thus a solution containing 40 weight percent of ammonium nitrate and in which the hydrogen peroxide-water portion contains 90 weight percent of  $H_2O_2$  has a freezing point of about -30° F. A so-called 80%  $H_2O_2$ -30%  $NH_4NO_3$  solution has a freezing point of below -70° F.

Concentrated aqueous hydrogen peroxide solutions have been used as monopropellants by catalytically decomposing the hydrogen peroxide using such catalysts as potassium permanganate or copper oxide. Since the decomposition products contain free-oxygen the monopropellant system is inefficient. However, fuels which are hypergolic with nitric acid oxidizers may be much less active or even inactive with concentrated  $H_2O_2$  solutions. Anhydrous hydrazine is usually considered to be the only fuel that is sufficiently hypergolic with concentrated  $H_2O_2$  solutions to be practical; however, hydrazine has the disability of a comparatively high freezing point. Some fuels are operative with  $H_2O_2$  solutions in the presence of a  $H_2O_2$  decomposition catalyst. Furthermore, the prior art fuels are less effective with ammonium nitrate containing aqueous hydrogen peroxide than with aqueous hydrogen peroxide alone.

An object of this invention is a method of generating gas by the hypergolic reaction of a fuel and a hydrogen peroxide oxidizer. Another object is a method of reaction propulsion by the hypergolic interaction of a fuel and a hydrogen peroxide oxidizer. Still another object is a method of reaction propulsion by the hypergolic interaction of a hydrogen peroxide oxidizer and a fuel which contains appreciable amounts of hydrocarbons, particularly non-hypergolic liquid hydrocarbons. A particular object is a method of generating gas by the hypergolic interaction of a defined fuel and an oxidizer consisting of an aqueous hydrogen peroxide solution containing dissolved ammonium nitrate. Another particular object is a method of rocket propulsion by the hypergolic interaction of a defined organic halothiophosphate and a defined hydrogen peroxide oxidizer when the temperature of the fuel and the oxidizer is above about -20° F. Other objects will become apparent in the course of the detailed description of the invention.

A method has been discovered for generating gas, which gas may be used as a substitute for compressed air for certain purposes or for driving the turbine of a jet engine or for rocket propulsion, which method comprises contacting

(1) A hypergolic fuel consisting essentially of a halothiophosphate selected from the class consisting of

(i) Aliphaticdihalothiophosphate containing from

55 1 to 6 carbon atoms and  
(ii) Dialiphatichalodithiophosphate containing from 2 to 8 carbon atoms and not more than 6 carbon atoms in one aliphatic radical and wherein the halogen radical is selected from the class consisting of chlorine and bromine, and

60 (2) An oxidizer selected from the class consisting of

(a) Aqueous hydrogen peroxide solutions which contain at least about 80 weight percent of  $H_2O_2$  and the remainder is essentially water and

65 (b) Aqueous hydrogen peroxide-inorganic salt solutions wherein the hydrogen peroxide-water portion contains at least about 80 weight percent of  $H_2O_2$ .

70 A mixed fuel made up of methylhalothiophosphate which contains as much as 40 volume percent of miscible hydrocarbon is hypergolic with aqueous hydrogen per-

oxide-ammonium nitrate solutions containing at least about 90 weight percent of hydrogen peroxide in the  $H_2O_2$ -water portion when the fuel and the oxidizer are at a temperature of about  $+60^\circ F$ . The lower the temperature of initial contact the less hydrocarbon tolerable in the mixed fuel.

Certain organic halothiophosphites ignite spontaneously when contacted with "hydrogen peroxide oxidizers." The various halothiophosphites do not have equal hypergolic activity with the same oxidizer. However, by proper selection of the halothiophosphate, it is possible to obtain a hypergolic reaction with a tolerable ignition delay when the halothiophosphate and the oxidizer are at a temperature of about  $-20^\circ F$ . at the moment of initial contact in the gas generating chamber.

These organic halothiophosphites have the generic empirical formula  $(RS)_aPX_b$ , where P represents the element phosphorus, S represents the element sulfur, X represents a halogen radical selected from the class consisting of chlorine and bromine, and R represents an aliphatic hydrocarbon radical, and wherein "a" is 1 or 2, "b" is 1 or 2 and the sum of "a" and "b" is 3.

The halothiophosphites which are suitable for the purposes of this invention contain aliphatic hydrocarbon radicals which may be paraffinic, e.g., methyl, ethyl, isopropyl and n-propyl; or olefinic, e.g., ethenyl, propenyl, isopropenyl, or acetylenic, e.g., ethynyl and propynyl; or cycloalkyl or cycloalkenyl, e.g., cyclopropyl and cyclopropenyl. In the case of the aliphaticdihalothiophosphites, the total number of carbon atoms should be not more than 6; while in the case of the dialiphatichalothiophosphites, the total number of carbon atoms should be not more than 8 and not more than 6 carbon atoms should be present in any one aliphatic radical.

The most suitable halothiophosphites for the purposes of this invention are the alkylhalothiophosphites wherein the alkyl radicals are selected from the group consisting of methyl, ethyl and mixtures thereof. For operation where the halothiophosphate and the oxidizer will be at a temperature of about  $-20^\circ F$ . at the moment of initial contacting of the halothiophosphate and the oxidizer, the preferred halothiophosphites are the methylhalothiophosphites.

A mixed fuel which is suitable for the generation of gas can be made by mixing aliphatichalothiophosphites with miscible hydrocarbons. The minimum amount of halothiophosphate necessarily present in said hypergolic mixed fuel will vary with the type of hydrocarbon, the desired temperature of operation and the type of  $H_2O_2$  oxidizer. For example: As much as 40% of a petroleum fraction is tolerable in a hydrocarbon-methylchlorothiophosphate blend which must be hypergolic at about  $+60^\circ F$ . when using an ammonium nitrate containing "90% hydrogen peroxide" oxidizer. In general petroleum hydrocarbon fractions are suitable materials as for example those fractions boiling between about  $300^\circ$  and  $600^\circ F$ . which correspond to the fuel requirement of military jet engines. Aromatic hydrocarbons which boil below about  $600^\circ F$ . are suitable hydrocarbons for this purpose. The hypergolic activity of the mixed fuel can be improved at lower atmospheric temperatures by using as the hydrocarbon component olefinic hydrocarbons such as thermally cracked naphthas and gas oils or turpentine. Conversely, at higher atmospheric temperatures a hypergolic mixed fuel containing less halothiophosphate is obtainable by the use of unsaturated hydrocarbons.

The oxidizers of this invention are either concentrated aqueous hydrogen peroxide solutions or aqueous hydrogen peroxide solutions containing dissolved inorganic salts, for example, ammonium halides, sodium sulfate, sodium nitrate, etc.; for low temperature operation requiring a short ignition delay, ammonium nitrate must be used as the salt. The concentrated aqueous hydrogen peroxide solutions should contain at least about 80 weight percent

of  $H_2O_2$ ; the remainder of the solution is essentially water.

The hypergolic activity of the aqueous hydrogen peroxide solution is improved by increasing the concentration of the peroxide. Commercially available 90%  $H_2O_2$  solution is an excellent oxidizer for operation above  $0^\circ F$ . For low temperature operation it is preferred to use aqueous  $H_2O_2$ -ammonium nitrate solutions, such as "90%—40%" or "80%—30%" solutions.

Concentrated aqueous hydrogen peroxide solution as made commercially is virtually only  $H_2O_2$  and water. In order to improve storage stability small amounts of stabilizers are commonly added to the solution, e.g., sodium stannate, tetrasodium pyrophosphate, adipic acid, 15 tartaric acid; in general only trace amounts of stabilizers are added so that the solution consists essentially of hydrogen peroxide and water.

In order to depress the freezing point of aqueous hydrogen peroxide solutions soluble inorganic salts are 20 dissolved therein, e.g., sodium nitrate, potassium nitrate and ammonium nitrate have been used. These salt-containing solutions are commonly designated in terms of the weight percent of salt in the total solution and the weight percent of hydrogen peroxide present in the aqueous portion of the solution, e.g., 90%  $H_2O_2$ —40%  $NH_4NO_3$  indicates that the total aqueous hydrogen peroxide-nitrate solution consists of 40 weight percent of ammonium nitrate and 60 weight percent of aqueous hydrogen peroxide composed of 90 weight percent of

25  $H_2O_2$  and the remainder essentially water. This particular solution has a freezing point of  $-30^\circ F$ . A temperature of  $-70^\circ F$ . is attainable with an 80%  $H_2O_2$ —30%  $NH_4NO_3$  solution. It is preferred to operate in the presence of ammonium nitrate because of the 30 pronounced favorable effect on the hypergolic activity of the fuels of this invention.

It has previously been found that trithiophosphites having the empirical formula  $RR'R''S_3P$  where R, R' and R'' represent aliphatic hydrocarbon radicals containing 40 from 1 to 3 carbon atoms and the total number of carbon atoms in the molecule is between 3 and 7 are hypergolic with the above defined  $H_2O_2$  oxidizers at temperatures above about  $0^\circ F$ . Examples of these fuels are trimethyltrithiophosphate and triethyltrithiophosphate. The 45 hypergolic activity of these fuels at lower temperatures can be greatly improved by adding thereto small amounts of the above defined halothiophosphites, i.e., the halothiophosphites have a synergistic catalytic effect on the activity of the aliphaticthiophosphites. For low temperatures the halothiophosphate-thiophosphate fuel should contain between about 1 and 20 volume percent of the halothiophosphate.

Ethylchlorothiophosphate was prepared by the method of Claesson, J. Prakt. Chem. (2), 15, 211 (1877), as 55 follows: Phosphorus trichloride (1 mol) was introduced into a 3-necked flask along with 100 ml. of  $CHCl_3$ . Ethyl mercaptan (1.38 mols) was added at  $0^\circ C$ . The reaction mixture was heated to about  $18^\circ C$ . and the temperature raised to  $50^\circ C$ . over a time of one hour. 60 The  $CHCl_3$  was distilled and the product was carefully fractionated through a Vigreux column about 5 inches tall at about 18 mm. Hg pressure. Two essentially pure products were obtained: ethyldichlorothiophosphate, boiling at  $77^\circ C$ . at 18 mm. Hg and diethylchlorothiophosphate, boiling at  $114^\circ C$ . at 18 mm. Hg.

The ignition characteristics of various fuels were 65 studied using a "drop" test. This method utilizes a test tube, 1 in. x 4 in., containing about 0.5 ml. of oxidizer. The fuel to be tested was drawn into a hypodermic syringe. It was then ejected forcibly against the oxidizer surface by depressing the syringe plunger. By this method amounts of fuel of as little as 0.01 ml. can be added. Low temperature tests were carried out by cooling the test tube and the oxidizer contained therein 70 by means of a bath; a drying tube inserted into the top

of the test tube excluded moisture. The fuel was cooled separately to the desired test temperature. By supercooling it was possible to carry out tests at temperatures below the freezing point of the fuel and/or the oxidizer.

The "ignition delay," which is the time elapsing between the addition of fuel to the oxidizer and visual ignition thereof, was determined as either (a) very short which corresponds to substantially instantaneous ignition, (b) short, which corresponds to substantially less than 1 second, and (c) more than 1 second, which time was determined by a stop watch.

The following tests illustrate the activity of the halo-thiophosphites of this invention and hydrazine with hydrogen peroxide oxidizers.

#### Test I

In order to observe the effectiveness of ethylchlorothiophosphites with oxidizers consisting of aqueous hydrogen peroxide and aqueous hydrogen peroxide-ammonium nitrate solutions, several runs were made at various temperatures using 0.5 ml. of oxidizer.

| Run No. | Fuel           | Fuel added, ml. | Oxidizer $H_2O_2$ — $NH_4NO_3$ , percent | Temp., °F. | Ignition delay, seconds |
|---------|----------------|-----------------|------------------------------------------|------------|-------------------------|
| 1       | Diethylchloro- | 0.10            | 80-30                                    | -22        | 54                      |
| 2       | do             | 0.10            | 80-30                                    | -50        | 105                     |
| 3       | do             | 0.05            | 90                                       | -10        | 35                      |
| 4       | do             | 0.05            | 90-40                                    | -10        | 24                      |
| 5       | do             | 0.04            | 90                                       | +70        | 1                       |
| 6       | Ethylchloro-   | 0.10            | 80-30                                    | -22        | 11                      |
| 7       | do             | 0.10            | 80-30                                    | -52        | 38                      |
| 8       | do             | 0.05            | 90                                       | +14        | 11                      |
| 8a      | do             | 0.05            | 90-40                                    | +14        | 2                       |

#### Test II

For comparative purposes hydrazine was contacted at various temperatures with various  $H_2O_2$  solutions as the oxidizer.

| Run No. | $H_2O_2$ , oxidizer, percent | Fuel added, ml. | Temp., °F. | Ignition delay               |
|---------|------------------------------|-----------------|------------|------------------------------|
| 9       | 90                           | 0.05            | +70        | Very short.                  |
| 10      | 80                           | 0.03            | +70        | Short.                       |
| 11      | 80                           | 0.10            | +14        | No ignition (effervescence). |
| 11a     | 90-40                        | 0.03            | +14        | No ignition.                 |
| 11b     | 90                           | 0.03            | +14        | Very short.                  |

#### Test III

The hypergolic activity of a mixture of thiophosphite and halo-thiophosphite was tested. Triethyltrithiophosphite prepared by reacting  $PCl_3$  and ethyl mercaptan was fractionated under conditions such that a trace amount of "chlorine" remained therein; believed to be diethylchlorodithiophosphite. The activity of this mixture was compared with chlorine-free triethyltrithiophosphite.

| Run No. | Fuel       | $H_2O_2$ , oxidizer, percent | Fuel added, ml. | Temp., °F. | Ignition delay |
|---------|------------|------------------------------|-----------------|------------|----------------|
| 12      | "Pure" do  | 90                           | 0.05            | +70        | No ignition.   |
| 13      | do         | 90                           | 0.06            | +70        | 77 sec.        |
| 14      | do         | 90                           | 0.08            | +70        | 22 sec.        |
| 15      | "Mixed" do | 90                           | 0.05            | +70        | 18 sec.        |
| 16      | do         | 90                           | 0.08            | +70        | 13 sec.        |

These runs show the favorable effect on ignition delay of a trace amount of the halo derivative on the activity of the trithiophosphite.

It is obvious from the data presented above that this invention can be used to generate gas at high pressure. This gas can be used for operating machinery such as "compressed air hammers" or for aircraft catapults; another important use for this high pressure gas is in the starting of the turbines of jet-type engines. The inven-

tion is particularly useful in aerial missiles which require a compact power plant that develops large amounts of energy over a very short period of time. Other examples of the use of this invention are: the rocket-assisted takeoff or flight of aircraft; aerial missiles; boosters for surface vehicles.

The relative proportion of oxidizer-to-fuel used will depend upon the type of operation, the temperature of operation and the type of fuel and oxidizer being used.

10 When using a 90%—40% hydrogen peroxide-ammonium nitrate solution as the oxidizer and methyldichlorothiophosphite as the fuel, between about 4 and 5 volumes of oxidizer are needed per volume of fuel.

By way of example this invention is applied to the 15 propulsion of a surface-to-air missile. The annexed figure which forms a part of this specification shows schematically the bipropellant feed system and the motor of this missile. This missile is suitable for operations wherein the fuel and the oxidizer can be maintained at

20 a temperature high enough to insure at least a short ignition delay, e.g., when using ammonium nitrate containing  $H_2O_2$  solution as the oxidizer and methyldichlorothiophosphite as the fuel, a temperature of about  $-20^{\circ}$  F.

In the drawing vessel 11 contains a quantity of gas 25 at high pressure; this gas must be inert with respect to the oxidizer and the fuel; suitable gases are nitrogen and helium. Herein helium is used as the inert gas. Helium from vessel 11 is passed through line 12 and through valve 13 which regulates the flow of gas to maintain a

30 constant pressure beyond valve 13. From valve 13 helium is passed through lines 14 and 16 into vessel 17 and simultaneously through line 18 into vessel 19.

Vessel 17 contains the oxidizer. Helium pressure forces the oxidizer out of vessel 17 through line 21 to 35 valve 22. Valve 22 is a solenoid actuated throttling valve.

Suitable electrical lines connect valve 22 to an electrical source and operating switch (not shown) at the control chamber at the launching site. The oxidizer is passed through line 23 and injector 24 into combustion chamber 40 26. Combustion chamber 26 is provided with an outlet nozzle 27.

Vessel 19 contains the fuel. Vessels 17 and 19 are constructed to withstand the high pressure imposed by the helium gas. The gas pressure forces fuel from vessel 19 through line 28 to solenoid actuated throttling valve 29.

45 Valve 29 is similar in construction and in actuation to valve 22. The fuel is passed through line 31 and injector 32 into combustion chamber 26.

Valves 22 and 29 are of such a size and setting that a 50 predetermined ratio of oxidizer-to-fuel is passed into combustion chamber 26. Injectors 24 and 32 are so arranged that the streams of oxidizer and fuel converge and contact each other forcibly, resulting in a very thorough intermingling of the fuel and the oxidizer.

55 The missile is launched by activating the solenoids on valves 22 and 29. In this example 4.5 volumes of oxidizer per volume of fuel is introduced into the combustion chamber. The oxidizer and the fuel react almost instantaneously upon contact in the combustion chamber; a large volume of very hot gas is produced in the combustion chamber, which gas escapes through orifice 27. The reaction from this expulsion of gas drives the missile toward its target.

Thus having described the invention, what is claimed is:

60 1. A method of generating gas, which method comprises injecting separately and essentially simultaneously into the combustion chamber of the gas generator (1) a hypergolic fuel consisting essentially of a member selected from the class consisting of (i) organicdihalo-thiophosphites containing not more than 6 carbon atoms and (ii) diorganichalodithiophosphites containing not more than 8 carbon atoms and not more than 6 carbon atoms in an organic group, wherein the organic group in (i) and (ii) above are aliphatic and the halogen radicals are selected

from the class consisting of chlorine and bromine and (2) an oxidizer selected from the class consisting of (a) aqueous hydrogen peroxide solutions consisting of at least about 80 weight percent of  $H_2O_2$  and the remainder essentially water and (b) aqueous hydrogen peroxide-ammonium nitrate solutions wherein the hydrogen peroxide-water portion is the predominant component and consists of at least about 80 weight percent of  $H_2O_2$  and the remainder essentially water, in an amount and at a rate sufficient to initiate a hypergolic reaction with and to support combustion of the fuel.

2. The method of claim 1 wherein said fuel is dimethylchlorodithiophosphate.

3. The method of claim 1 wherein said fuel is methyl-dichlorothiophosphate.

4. The method of claim 1 wherein said fuel is diethyl-chlorodithiophosphate.

5. The method of claim 1 wherein said fuel is ethylchlorothiophosphate.

6. The method of claim 1 wherein said oxidizer consists of about 80 weight percent of  $H_2O_2$  and the remainder essentially water.

7. The method of claim 1 wherein said oxidizer consists of about 90 weight percent of  $H_2O_2$  and the remainder essentially water.

8. The method of claim 1 wherein said oxidizer consists of a solution of hydrogen peroxide, water and ammonium nitrate, wherein the nitrate content is about 30 weight percent and the hydrogen peroxide-water portion consists of about 80 weight percent of  $H_2O_2$  and the remainder essentially water.

9. The method of claim 1 wherein said oxidizer consists of a solution of hydrogen peroxide, water and ammonium nitrate, wherein the nitrate content is about 40 weight percent and the hydrogen peroxide-water portion consists of about 90 weight percent of  $H_2O_2$  and the remainder essentially water.

10. A method of generating gas, which method comprises injecting separately and essentially simultaneously into the combustion chamber of the gas generator (1) a hypergolic mixed fuel consisting essentially of (I) a liquid miscible hydrocarbon and (II) methylchlorothiophosphate and (2) an oxidizer selected from the class consisting of (a) aqueous hydrogen peroxide solutions consisting of at least about 80 weight percent of  $H_2O_2$  and the remainder essentially water, and (b) aqueous hydrogen peroxide-ammonium nitrate solutions wherein the hydrogen peroxide-water portion is the predominant component and consists of at least about 80 weight percent of  $H_2O_2$  and the remainder essentially water, in an amount and at a rate sufficient to initiate a hypergolic reaction with and to support combustion of the mixed fuel.

11. The method of claim 10 wherein said hydrocarbon is a liquid petroleum fraction boiling between about 300° and about 600° F.

12. The method of claim 10 wherein said hydrocarbon is a liquid aromatic hydrocarbon boiling below about 600° F.

13. The method of claim 10 wherein said hydrocarbon is a liquid olefin boiling below about 600° F.

14. A method of generating gas, which method comprises injecting separately and essentially simultaneously into the combustion chamber of the gas generator (1) a hypergolic mixed fuel consisting essentially of (I) a liquid miscible hydrocarbon and (II) ethylchlorothiophosphate and (2) an oxidizer selected from the class consisting of (a) aqueous hydrogen peroxide solutions consisting of at least about 80 weight percent of  $H_2O_2$  and the remainder essentially water, and (b) aqueous hydrogen peroxide-ammonium nitrate solutions wherein the hydrogen peroxide-water portion is the predominant component and consists of at least about 80 weight percent of  $H_2O_2$  and the remainder essentially water, in an amount and at a rate sufficient to initiate a hypergolic reaction with and to support combustion of the mixed fuel.

15. A method of gas generation, which method comprises injecting separately and essentially simultaneously into the combustion chamber of the gas generator (1) a hypergolic fuel consisting essentially of (A) trialkyltrithiophosphites wherein the alkyl radicals contain from 1 to 3 carbon atoms and the total number of carbon atoms in the trithiophosphate is from 3 to 7 and (B) between about 1 and about 20 volume percent based on fuel of a halothiophosphate selected from the class consisting of (i) organic dihalothiophosphites containing not more than 6 carbon atoms and (ii) diorganichalothiophosphites containing not more than 8 carbon atoms and not more than 6 carbon atoms in an organic group, wherein the organic groups in (i) and (ii) above are aliphatic and the halogen radicals are selected from the class consisting of chlorine and bromine and (2) an oxidizer selected from the class consisting of (a) aqueous hydrogen peroxide solutions consisting of at least about 80 weight percent of  $H_2O_2$  and the remainder essentially water and (b) aqueous hydrogen peroxide-ammonium nitrate solutions, wherein the hydrogen peroxide-water portion is the predominant component and consists of at least about 80 weight percent of  $H_2O_2$  and the remainder essentially water, in an amount and at a rate sufficient to initiate a hypergolic reaction with and to support combustion of the fuel.

16. The method of claim 15 wherein said halothiophosphate is methyldichlorothiophosphate.

17. The method of claim 15 wherein said halothiophosphate is ethyldichlorothiophosphate.

18. The method of claim 15 wherein said trithiophosphate is trimethyltrithiophosphate.

19. The method of claim 15 wherein said trithiophosphate is triethyltrithiophosphate.

#### References Cited in the file of this patent

#### FOREIGN PATENTS

257,649 Switzerland \_\_\_\_\_ May 2, 1949

#### OTHER REFERENCES

Claesson: "J. Prakt. Chem.", vol. 15 (1877), page 211.